# EUROPEAN PATENT SPECIFICATION

(11) **EP 1 880 056 B1**
(45) Date of publication and mention of the grant of the patent: **01.04.2009**
(21) Application number: 06733387.2
(22) Date of filing: 03.05.2006
(51) Int. Cl.: D21H 11/22, C08J 5/06, D06M 11/77

(54) **FREE CLAY-COATED CELLULOSIC FIBERS FOR COMPOSITES AND A METHOD OF PRODUCING THEM**
FREIE TONBESCHICHTETE CELLULOSEFASER FÜR VERBUNDWERKSTOFFE UND HERSTELLUNGSVERFAHREN DAFÜR
FIBRES DE CELLULOSE LIBRES POUR COMPOSITES ENDUITES DE KAOLIN ET PROCEDE DE PRODUCTION ASSOCIE

(30) Priority: 12.05.2005 SE 0501075
(43) Date of publication of application: 23.01.2008
(73) Proprietor: KORSNÄS AB, S-801 81 Gävle (SE)
(72) Inventor: BANKE, Karl, S-271 42 Ystad (SE); LINDSTRÖM, Tom, S-192 72 Sollentuna (SE)
(74) Representative: Nilsson, Brita Linnea
(86) International application number: PCT/SE2006/000532
(87) International publication number: WO 2006/121385

(56) References cited:
- EP-A2- 0 288 070
- WO-A1-97/00838
- GB-A- 480 740
- GB-A- 2 019 461

## Description

The present invention relates to free clay-coated cellulosic fibers and a method of producing such fibers. The fibers are particularly useful as components in composites. The free fibers are in a dry state readily dispersed into e.g. thermoplastic polymers enabling a uniform distribution of the fibers in the resulting composite.

### Background.

Composite materials are manufactured to replace traditional structural materials with lighter and cheaper products and at the same time keep the good mechanical properties inherent in the traditional structural materials. Fibers are introduced into a polymer matrix to increase the strength and stiffness of such a composite.

The predominant matrix for composite materials has been thermosetting resins because of their hardness, stiffness, and thermo-stability. Thermoplastic polymer matrices have the advantage of short process time, good storability, lack of chemical reaction, and that they are easy to reprocess. This has led to an increasing use of thermoplastic materials as a composite matrix, e.g. polypropylene.

Common reinforcements used for composite materials are carbon fibers, fiberglass or other inorganic fibers. However, organic fibers, such as cellulosic fibers, are gaining importance, mainly because of their low density, high strength, low cost, and that they come from renewable resources.

The hydrophilic nature of the cellulosic fibers causes problems when introduced into a hydrophobic polymer matrix. The interaction between the matrix and the cellulosic fibers is poor, which leads to a weak adhesion. Inadequate adhesion can lead to de-bonding, internal strains and porosity, which in turn lead to a weaker material.

Another complication with the hydrophilic fibers is their ability to absorb moisture and water. The swelling of the fibers can cause problems with dimensional stability and introduce stress concentrations in the composite. The water can also cause problems with the compounding of the composite material. Since the compounding process using thermoplastic polymers occurs at temperatures around 200 °C, the water will be evaporated and cause cavities and cracks in the product.

The dispersion of the fibers in the matrix is also an important factor when it comes to mechanical properties and appearance. It is assumed that maximum strength and stiffness will be achieved when the strength of every single fiber is utilized. However, cellulosic fibers have a tendency to flocculate due to the strong fiber-fiber joints formed when the pulp is dried. It is also difficult to disperse hydrophilic fibers in an olefinic matrix such as polyethylene or polypropylene.

GB-A-2019461 discloses cellulose fibers that are individually clad with finely divided inorganic material, preferably clay.

### Description of the invention

The present invention provides a method of producing free clay-coated cellulosic fibers suitable for dispersion into a composite matrix. The clay-coating makes it easier to produce free fibers during defibration and to disperse the fibers into the polymer matrix when the composite material is compounded, since the clay acts as a blocking agent on cellulosic fibers preventing the fibers from aggregating during formation of the fiber network and thus preventing the development of strong fiber-fiber joints.

Thus, one aspect of the invention is directed to a method of producing free clay-coated cellulosic fibers, which method comprises the following steps:
a) mixing an aqueous cationic polyelectrolyte solution and an aqueous suspension of cellulosic fibers to render a positive surface charge to the fibers,
b) adding an aqueous slurry of swollen exfoliated clay flakes or swollen homogenized clay particles having an average particle size in the range of 0.4 - 1.6 µm to the mixture of a) to coat the charged fibers with the clay flakes or the clay particles,
c) dewatering and drying the mixture of b) to yield a mass of clay-coated fibers having a dry solids content of 85 to 95%,
d) transporting the mass of c) to a defibrator where the mass is defibrated to yield free clay-coated cellulosic fibers.

The drying of the fibers to a dry solids content of 85 to 95 % is made of practical reasons since the humidity of air would not allow a dryer fiber mass to be transported to a defibrator without special arrangements.

In an embodiment of this aspect of the invention the mixture of a) is filtered to remove excess cationic polyelectrolyte and the surface charged fibers are resuspended in water prior to the step b).

In a preferred embodiment the free clay-coated cellulosic fibers produced in d) are dried to a dry solids content exceeding 95%. The dryer the clay-coated fibers are, the better they are as components in a composite. The drying of the free clay-coated cellulosic fibers to a dry solids content exceeding 95% may be effected simultaneously with mixing the fibers with a polymer matrix at elevated temperature prior to compounding.

In another embodiment of the invention the clay is bentonite, in particular montmorillonite.

Another aspect of the invention is directed to free clay-coated cellulosic fibers, wherein the fibers have a coating of exfoliated clay flakes or clay powder having an average particle size of 0.4 - 1.6 µm (as determined by Mastersizer MS 20 (Malvern Instruments, UK) and a dry solids content exceeding 95%.

In an embodiment of the invention the coating covers 10 - 90 % of the fiber surfaces. The amount of clay needed to achieve this coverage is approximately 1 - 40 mg/g of fibers.

The free clay-coated cellulosic fibers according to the invention or produced according to the invention are, in a preferred embodiment, for use as components in composite materials, and the composite materials preferably comprise the free clay-coated cellulosic fibers dispersed in a thermoplastic polymer.

Yet another aspect of the invention is directed to the use of free clay-coated cellulosic fibers according to the invention or produced according to the invention as components in composite materials.

In an embodiment of this aspect of the invention, the composite material comprises the free clay-coated cellulosic fibers dispersed in a thermoplastic polymer.

The cellulosic fibers that can be used in the present invention include all types of wood-based fibers, such as bleached, half-bleached and unbleached sulphite, sulphate-and soda pulps, together with bleached, half-bleached and unbleached mechanical, thermo-mechanical, chemo-mechanical, and chemo-thermo-mechanical pulps, and mixtures of these. Both new fibers and recycled fibers can be used in the present invention, as can mixtures of these. Pulps from both softwood and hardwood trees can be used, as can mixtures of such pulps. Pulps that are not based on wood, such as cotton linters, regenerated cellulose, kenaf and grass fibers may also be used in the present invention.

To the fiber surface a cationic polyelectrolyte is adsorbed in the method of the invention. It is intended throughout the present description and claims that the expression "polyelectrolyte" includes all kinds of polyelectrolytes, such as quaternized and unquaternized copolymers of dimethylamino ethyl (or methyl) methacrylate/methacrylamide or 3-acrylamide-3-methylbutyl tri(di)methylammonium chloride and acrylamide, polyethyleneimines, dimethylamine-epichlorohydrin polymers, ethyleneimine grafted polyamidoamines, polyamidoamineepichlorohydrin polymers, ethyleneimine grafted polyacrylates, Mannich type formaldehyde/dimethylamine polyacrylamide adducts, and homo- and co-polymers (with acrylamide) of diallydimethylammonium chloride.

Further, it is intended throughout this description and claims that the expression "clay" embraces all kinds of laminated silica minerals in their swellable form e.g. Na⁺-form, such as bentonite, preferably montmorillonite clay which is a negatively charged inorganic clay (Al₂Si₄O₁₀(OH)₂*nH₂O) stacked in layers. The clay is in this invention used swollen and homogenized or delaminated or exfoliated, which in this description refers to the operation of mechanically, chemically or in any other way separate the thin layers in the mineral "stacks" or "aggregates" from each other. The mechanical treatment can be performed in a high-pressure homogenizer, microfluidizer, sand grinder, ball or pebble mills, extruders or rotor-stator colloid mills, or any other suited device. The result is an aqueous slurry with small and thin mineral particles, platelets or flakes.

The composite materials in which the free clay-coated cellulosic fibers of the invention, or produced by the invention, are dispersed additionally comprise a matrix that can be any suitable thermoplastic polymer, such as polyolefins (e.g. polyethylene, polypropylene), polyvinyls (e.g. polyvinyl chloride and polyvinyl acetate), polystyrene, polyimides, polyamides, polyacrylates, ABS polymers, silicone resins, polyurethane resins, polylactic acid, poly(lactic-co-glycolic acid), and polysaccharides (e.g. cellulose based polymers). In the examples poly-diallyldimethylammonium chloride is used as the cationic polyelectrolyte.

The invention will now be further illustrated by reference to the drawings and the examples, but it should be understood that these specific disclosures do not limit the scope of the invention defined by the appended claims.

### Short description of drawings

**Fig.1** is a diagram showing the adsorption isotherm of clay on pulp in a paper mill process water.
**Fig. 2** is a picture of a composite film containing untreated fibers. The film is scanned over 20 x 8 cm.
Fig. 3 is a picture of a composite film containing fibers with 1 mg/g clay adsorbed. The film is scanned over 20 x 8 cm.

### Examples

### Example 1.

### Adsorption of exfoliated clay onto fibers

This example illustrates the deposition of montmorillonite clay onto a fiber surface.

To a mixture of bleached northern softwood fibers taken after the last bleaching step and a process water from a paper mill, at a concentration of 0.5 %, 1.5 mg/g poly-DADMAC (poly-diallyldimethylammonium chloride), Alcofix 110 (CDM, Västra Frölunda, Sweden) was added. The mixture was stirred for 30 minutes and then filtered through a size 3 filter paper (Munktell). The fibers were then divided into six equally large portions and added to process water at a concentration of 0.5 %. To these six samples, different amounts of exfoliated montmorillonite clay (Hydrocol MD (CDM); 5, 10, 20, 30, 40 and 50 mg/g) was added and they were stirred for 10 minutes. Before the clay was added to the fiber suspensions it was swollen in deionized water for 24 hours at a concentration of 20 g/l. The clay was then homogenized in a high-pressure homogenizer, Mini-lab type 8.30H (APV Homogeniser group), followed by centrifugation at 3600 g and 15 minutes in a Multifuge 3L Heraeus (Kendro Laboratory Products, Germany). The clear aqueous phase, with a clay concentration of 12.76 g/I, was collected and used.

The average size of the clay particles retrieved from the homogenizer was determined with a Mastersizer MS20 and a 45 mm lens (Malvern Instruments, UK) to be in the range of 0.4 - 1.6 µm.

After the clay addition, the fibers were filtered through dry weighed filter papers and the amount of clay not adsorbed onto the fibers was measured by a charge reversal experiment (Mütek PCD 03-titrator). The fibers were dried over night and weighed so that an exact amount of fibers used was obtained. The result is shown in Figure 1.

### Example 2.

### ESCA

This example illustrates the surface coverage obtained when the clay was adsorbed.

Three fiber samples with different amounts of exfoliated clay adsorbed (2,10, and 20 mg/g), one sample with clean fibers, and one clay sample were all subjected to ESCA (Electron Spectroscopy for Chemical Analysis). The method measures the different amounts of chemical elements present at the surface of the sample (5-10 nm deep). The elements of interest for this project were Si, Al and C. The aim of the analysis was to investigate how much of the fiber surface that could be covered with the clay. The analysis was performed on an AXIS Integrated Imaging XPS.

The surface coverage of the exfoliated clay was calculated from the ESCA results by taking the ratio of Si/(Si+C3) where C3 is the signal from the carbon in O-C-O present only in the cellulose chain. As shown in Table 1, the surface coverage increases with increasing amount of clay attached. A 75 % coverage of the fiber surface was achieved when 20 mg/g clay had been adsorbed onto the fibers.

**Table 1. The clay surface coverage of the fibers calculated from the ESCA results.**

| **Adsorbed Amount of Clay [mg/g]** | **Surface Coverage [%]** |
|---|---|
| 2 | 11 |
| 10 | 53 |
| 20 | 75 |

### Example 3

### Compounding of Fiber-Polymer Composite

### Mixing Fibers and Matrix

In an attempt to make the fibers homogenously distributed throughout the polymer matrix, the free clay-coated fibers produced according to the invention and polypropylene pellets were mixed in the solid state. Five different batches of fibers with different amounts of clay adsorbed and one batch with untreated fibers were mixed: After drying the fibers and the pellets over night at 90°C, they were blown through a ventilation tube for five minutes. The device was a modified blower from AB Johanssons Chuckfabrik in Bredaryd (model GK 20-E). The pellets were somewhat integrated in the mass of free fibers which should simplify the distribution of the fibers in the coming compounding.

After the "dry" mixing, the fibers and pellets were fed into a Buss co-kneader extruder, which held the temperatures 175, 180, 180, and 190°C in the different heating sections. A string of fiber composite was extruded and then granulated in a pelletizer (H. Dreher, Maschinenbau, D-51 Aachen, SG10 Ni). The composite pellets were once more fed into the co-kneader extruder and the pelletizer to more evenly distribute the fibers in the polymer matrix.

### Extrusion

The composite pellets were fed into a Brabender Compact extruder (19mm/25d screw, 40 rpm, 195, 210, 210, 210 °C). Films were extruded through an 80 mm wide and 0,8 mm thick slit. The films were later optically analyzed.

### Example 4.

### Optical analysis of composites

This example illustrates the improvement in dispersion accomplished by adsorbing a polyelectrolyte and flaky clay.

In order to see how well the fibers were dispersed in the matrix, the extruded films were placed in an Epson Expression 1680 Pro scanner. The samples were penetrated with light making fiber flocks appear as dark spots. The films were scanned over an area of 20 x 8 cm with 16-bit grayscale, 300 dpi. The pictures were edited with Adobe Photoshop 3.0. A threshold value of 113 (grayness level from 0-255 where 0 is black) was applied making areas over this value white and areas under it black. This value was chosen because it eliminated most of the smallest dots, leaving the larger fiber flocks more visible.

Examples of pictures-from the composite film scanning are shown in Fig.-2. (composite film containing untreated fibers) and Fig. 3 (composite film containing fibers with 1 mg/g clay adsorbed). The amount of dark spots, i.e. areas with fiber flocks, is an indication of how well the cellulosic fibers are dispersed in the polymer matrix.

As shown in Figs. 2 and 3, the fiber flocks visible in Fig. 2 are almost completely eliminated in Fig. 3. These films are extruded in the same manner and at equal humidity.

From the comparison of the Figs. 2 and 3 it can be concluded that the composite containing untreated cellulose fibers contained aggregates of fibers (dark dots), whereas the composite containing free clay-coated cellulose fibers of the invention have these uniformly distributed in the composite (no dark dots).

## Claims

1. A method of producing free clay-coated cellulosic fibers comprising the steps of
a) mixing an aqueous cationic polyelectrolyte solution and an aqueous suspension of cellulosic fibers to render a positive surface charge to the fibers,
b) adding an aqueous slurry of swollen exfoliated clay flakes or swollen homogenized clay particles having an average particle size in the range of 0.4 - 1.6 µm to the mixture of a) to coat the charged fibers with the clay flakes or the clay particles,
c) dewatering and drying the mixture of b) to yield a masse of clay-coated fibers having a dry solids content of 85 to 95%,
d) transporting the mass of c) to a defibrator where the mass is defibrated to yield free clay-coated cellulosic fibers.

2. The method according to claim 1, wherein the mixture of a) is filtered to remove excess cationic polyelectrolyte and the surface charged fibers are resuspended in water prior to the step b).

3. The method according to claim 1 or 2, wherein the free coated cellulosic fibers produced in d) are dried to a dry solids content exceeding 95%.

4. The method according to any one of the claims 1 - 3, wherein the clay is bentonite.

5. The method according to claim 4, wherein the bentonite is montmorillonite.

6. Free clay-coated cellulosic fibers, wherein the fibers have a coating of exfoliated clay flakes or clay powder having an average particle size of 0.4 - 1.6 µm and a dry solids content exceeding 95%.

7. Free clay-coated cellulosic fibers according to claim 6, wherein the coating covers 10 - 90 % of the fiber surfaces.

8. Free clay-coated cellulosic fibers according to claim 6 or 7 or produced according to any one of claims 1 -5 for use as components in composite materials.

9. Free clay-coated cellulosic fibers according to claim 8, wherein the composite material comprises the free clay-coated cellulosic fibers dispersed in a thermoplastic polymer.

10. Use of free clay-coated cellulosic fibers according to claim 6 or 7 or produced according to any one of claims 1 -5 as components in composite materials.

11. Use according to claim 10, wherein the composite material comprises the free clay-coated cellulosic fibers dispersed in a thermoplastic polymer.

## Patentansprüche

1. Verfahren zur Herstellung von freien tonbeschichteten Cellulosefasern, umfassend die Schritte:
a) Mischen einer wäßrigen Lösung eines kationischen Polyelektrolyten und einer wäßrigen Suspension von Cellulosefasern, um auf den Fasern eine positive Oberflächenladung aufzubringen,
b) Zugeben einer wäßrigen Aufschlämmung von gequollenen, abgeblätterten Tonflocken oder gequollenen homogenisierten Tonpartikeln mit einer mittleren Partikelgröße im Bereich von 0,4 bis 1,6 µm zu der Mischung aus a), um die geladenen Fasern mit Tonflocken oder Tonpartikeln zu beschichten,
c) Entwässern und Trocknen der Mischung aus b), um eine Masse von tonbeschichteten Fasern mit einem Trockenfeststoffgehalt von 85 bis 95 % zu erhalten,
d) Transportieren der Masse aus c) zu einem Zerfaserer, worin die Masse zerfasert wird, um freie tonbeschichtete Cellulosefasern zu erhalten.

2. Verfahren gemäß Anspruch 1, worin die Mischung aus a) filtriert wird, um überschüssigen kationischen Polyelektrolyten zu entfernen und die auf der Oberfläche geladenen Fasern vor dem Schritt b) in Wasser re-suspendiert werden.

3. Verfahren gemäß Anspruch 1 oder 2, worin die in d) herbestellten freien beschichteten Cellulosefasern auf einen Trockenfeststoffgehalt getrocknet werden, der 95 % überschreitet.

4. Verfahren gemäß irgendeinem der Ansprüche 1 bis 3, worin der Ton Bentonit ist.

5. Verfahren gemäß Anspruch 4, worin das Bentonit Montmorillonit ist.

6. Freie tonbeschichtete Cellulosefasern, worin die Fasern eine Beschichtung aus abgeblätterten Tonflocken oder Tonpulver mit einer mittleren Partikelgröße von 0,4 bis 1,6 µm und einen Trockenfeststoffgehalt größer 95 % aufweisen.

7. Freie tonbeschichtete Cellulosefasern gemäß Anspruch 6, worin die Beschichtung 10 bis 90 % der Faseroberfläche bedeckt.

8. Freie tonbeschichtete Cellulosefasern gemäß Anspruch 6 oder 7 oder hergestellt gemäß irgendeinem der Ansprüche 1 bis 5 zur Verwendung als Komponenten in Kompositmaterialien.

9. Freie tonbeschichtete Cellulosefasern gemäß Anspruch 8, worin das Kompositmaterial die freien tonbeschichteten Cellulosefasern dispergiert in einem thermoplastischen Polymer umfaßt .

10. Verwendung der freien tonbeschichteten Cellulosefasern gemäß Anspruch 6 oder 7 oder hergestellt gemäß irgendeinem der Ansprüche 1 bis 5 als Komponenten in Kompositmaterialien.

11. Verwendung gemäß Anspruch 10, worin das Kompositmaterial die freien tonbeschichteten Cellulosefasern dispergiert in einem thermoplastischen Polymer umfaßt.

## Revendications

1. Procédé de production de fibres de cellulose libres enduites d'argile comprenant les étapes de
a) mélanger une solution de polyélectrolyte cationique aqueuse et une suspension aqueuse de fibres de cellulose pour donner une charge de surface positive aux fibres,
b) ajouter une boue aqueuse de flocons d'argile exfoliés gonflés ou de particules d'argile homogénéisées gonflées d'une taille de particules moyenne dans la plage de 0,4-1,6 µm au mélange de a) pour revêtir les fibres chargées avec les flocons d'argile ou les particules d'argile,
c) éliminer l'eau et sécher le mélange de b) pour obtenir une masse de fibres revêtues d'argile ayant une teneur en matières solides sèches de 85 à 95%,
d) transporter la masse de c) à un défibrateur où la masse est défibrée pour obtenir des fibres de cellulose libres revêtues d'argile.

2. Procédé selon la revendication 1, où le mélange de
a) est filtré pour retirer des polyélectrolytes cationiques excédentaires, et les fibres chargées en surface sont resuspendues dans l'eau avant l'étape b).

3. Procédé selon la revendication 1 ou 2, où les fibres de cellulose libres revêtues produites dans d) sont séchées à une teneur en matières sèches dépassant 95%.

4. Procédé selon l'une quelconque des revendications 1 à 3, où l'argile est la bentonite.

5. Procédé selon la revendication 4, où la bentonite est la montmorillonite.

6. Fibres de cellulose libres revêtues d'argile, où les fibres ont un revêtement de flocons d'argile exfoliés ou de poudre d'argile ayant une taille de particules moyenne de 0,4-1,6 µm et une teneur en matières sèches dépassant 95%.

7. Fibres de cellulose libres revêtues d'argile selon la revendication 6, où le revêtement couvre 10-90% des surfaces des fibres.

8. Fibres de cellulose libres revêtues d'argile selon la revendication 6 ou 7 ou produites selon l'une quelconque des revendications 1 à 5 pour utilisation comme composants dans des matériaux composites.

9. Fibres de cellulose libres revêtues d'argile selon la revendication 8, où le matériau composite comprend les fibres de cellulose libres revêtues d'argile dispersées dans un polymère thermoplastique.

10. Utilisation de fibres de cellulose libres revêtues d'argile selon la revendication 6 ou 7 ou produites selon l'une quelconque des revendications 1 à 5 comme composants dans des matériaux composites.

11. Utilisation selon la revendication 10, où le matériau composite comprend les fibres de cellulose libres revêtues d'argile dispersées dans un polymère thermoplastique.
